

## UNITED STATES PATENT OFFICE

2,142,720

## MANUFACTURE OF ARTIFICIAL MATERIALS

Henry Dreyfus, London, and Robert Wighton Moncrieff and Frank Brentnall Hill, Spondon, near Derby, England, assignors to Celanese Corporation of America, a corporation of Delaware

No Drawing. Application November 19, 1936, Serial No. 111,596. In Great Britain February 2, 1934

5 Claims. (Cl. 117—2)

This invention relates to improvements in the manufacture of artificial materials and particularly to improvements in the manufacture of yarns, especially yarns having a basis of cellulose acetate or other organic derivative of cellulose, and is a continuation in part of our application S. No. 4,510 filed February 1, 1935.

The cellulose derivative artificial yarns which are employed commercially for the production of normal plain fabrics have, in general, a twist of about 2 to 5 turns per inch, while yarns having somewhat higher twist, for example 10 to 15 up to about 20 turns per inch, may be employed for the production of particular kinds of fabrics, for example voile fabrics. It has now been discovered that artificial yarns may be stretched in the presence of hot aqueous fluid, which may be steam or hot water, e. g., by 15-40 or 50% up to 100% or more of their original length, and twisted in a single operation, and yarns of relatively low twist (i. e., up to about 20 turns per inch) and of increased tenacity may be obtained.

The filaments twisted according to the present invention may have been obtained from cellulose derivative solutions, or have been produced by a process of esterification or etherification without loss of structure, e. g. by acetylation of continuous filaments of regenerated cellulose in the presence of benzene or other suitable non-solvent. They may contain delustring or loading agents, e. g., barium sulphate, titanium dioxide, stannic phosphate or diacetox benzidine, and may have been subjected to stretching and/or shrinking operations, e. g. as described in U. S. applications S. Nos. 4,510 filed February 1, 1935, 4,511 filed February 1, 1935 and 611,240 filed May 13, 1932. Again, the filaments may be saponified, e. g., partially saponified throughout their cross-section or superficially saponified.

40 The steam employed in the process of the present invention may be saturated or wet steam and may be at temperatures of the order of 95 to 100° C. or 105° C., e. g. at a temperature corresponding to a super-atmospheric pressure of 1 to 5 or 10 cm. of water, or at higher temperatures, for example 110°, 120° C. or up to 140° C. or more, corresponding to pressures of 10, 15 or 20 up to 30 pounds per square inch or more above atmospheric pressure.

50 The combined stretching and twisting operation may be effected by means of the apparatus described in British specification No. 440,653, wherein the steaming chamber for the yarn consists of a short tube offset from a main steam supply pipe.

A method of carrying out the process of the present invention which has been found particularly valuable consists in drawing a yarn having no twist or only a very low twist, for example 0.5 or 1 turn per inch, from a bobbin which is rotating at a high speed, for example 3000, 5000, 11,000, 18,000 or more revolutions per minute, through a substantially closed steam chamber 5 and then taking it up on a bobbin rotating at a suitable speed, which will depend inter alia on 10 the speed of rotation of the supply bobbin and on the number of turns per inch which it is desired to insert in the yarn. In this process a tension is exerted on the yarn which, on account of the action of the steam on the yarn, stretches 15 it to a degree which will depend upon the steaming conditions. In general the higher the temperature of the steam the greater will be the stretch produced. For example by drawing a cellulose acetate yarn of about 150 denier from 20 a supply bobbin rotating at 11,000 revolutions per minute into and out of a steaming chamber of about 3 inches in length and taking it up at a speed of about 140 metres per minute a stretch corresponding to a reduction in denier of from 25 150 to about 130 may be produced with wet steam at a pressure of about 10 pounds gauge, while with wet steam at a pressure of about 30 pounds gauge the denier may be reduced to 30 about 100-110. By this means a yarn of increased tenacity having a twist of about 2 turns per inch may be obtained.

Higher degrees of twist may be inserted. For example cellulose acetate yarn having a twist of 35 12 to 14 turns per inch and a considerably increased tenacity may be obtained by means of an apparatus similar to that illustrated in British specification No. 440,653, using 9-inch tubes offset from a main steam pipe and containing wet steam at a pressure of about 5-10 pounds per 40 square inch above atmospheric pressure, the spindle speeds being 6000-7000 revolutions per minute.

The length of the steam chamber yielding the best results will depend inter alia upon the take-up speed of the yarn and may, e. g., be 3 inches 45 or 6 inches up to 18 inches or more. In general it appears that the greater the take-up speed the longer should be the path of the yarn through the steam, provided that the other conditions remain the same. For example, while, using a supply 50 bobbin rotating at about 5000 revolutions per minute, good results may be obtained with a 3 inch steam chamber at a pressure of 30 pounds per inch and a take-up speed of about 60 metres per minute, it is found that better results are, 55

in general, obtained by the use of a steaming chamber of about 6 inches in length, the other conditions being the same. On the other hand, with a longer steam chamber the steam temperature may in general be reduced to obtain similar results.

Another method of carrying out the process of the present invention consists in feeding yarn from a dry spinning apparatus, a bobbin or other source, through a steaming chamber and taking it up on a winding and twisting device, e. g., a ring or cap spinning apparatus.

If it is desired to increase the degree of stretch produced according to the process of the present invention, the tension may be increased, e. g. by inserting a gate or similarly acting device in the path of the yarn. Thus a bundle of filaments may be drawn from a rapidly rotating bobbin through a floating ring device as described in 20 U. S. Patent No. 1,784,581, then through a steam chamber and finally taken up on a bobbin or the like.

The process of the present invention may also be carried out using hot water instead of steam. 25 For example the yarn may be drawn off from a rotating bobbin and passed upwards through a small hole in a suitable receptacle containing hot water, and thence to a winding device. The hole may be provided with means adapted to lead 30 away any liquid issuing from the hole and prevent it from reaching the rotating bobbin. If desired the hole may take the form of a tube of fine bore fixed in the receptacle whereby the flow of liquid at the entrance of the thread may be 35 reduced. Again, hot water may be supplied to the yarn by passing it in contact with a horizontal roller, preferably circumferentially grooved, arranged to rotate in a bath of hot water and so carry water to the thread. Water may be used 40 at temperatures of 95 or 100° C. or at temperatures considerably higher, as for example 110-130 or 140° C. or more. At temperatures above the boiling point the water is employed under pressure in a substantially closed chamber, and even when 45 working at the boiling point or at temperatures below the boiling point it is preferable to use such a chamber.

Yarns made of cellulose acetate or other organic ester of cellulose which have been twisted 50 and stretched according to the process of the present invention may be partially or completely saponified, for example with caustic soda or other inorganic base, or with organic bases, for example methylamine or ethylene diamine, as described in U. S. applications S. Nos. 329 filed January 4, 1935, 752,376 filed November 9, 1934 and 756,285 filed December 6, 1934. Organic bases, and inorganic bases such as sodium silicate, are particularly useful when it is desired to 55 effect deep-seated saponification.

The process of the present invention is of particular value in the stretching and twisting of artificial filaments having a basis of cellulose acetate and especially cellulose acetate having an 60 acetyl value of about 52 to 56%. It may, how-

ever, also be employed in the stretching and twisting of other artificial filaments, for example continuous filaments having a basis of organic esters of cellulose other than cellulose acetate, such as cellulose formate, cellulose propionate, cellulose butyrate and cellulose nitro-acetate, cellulose ethers, for example methyl, ethyl and butyl celluloses, and cellulose ether-esters, for example ethyl cellulose acetate and oxy-ethyl cellulose acetate, and filaments having a basis 10 of regenerated cellulose.

Having described our invention what we desire to secure by Letters Patent is:

1. Process for the production of low twist yarn of improved tenacity, which comprises stretching 15 a yarn having a basis of an organic derivative of cellulose by at least 40% of its original length by passing it through hot aqueous fluid at a temperature of at least 95° C. during its travel between feed and take-up devices which insert a 20 low twist in the yarn, the stretching and twisting of the yarn being effected in the presence of the hot aqueous fluid.

2. Process for the production of low twist yarn of improved tenacity, which comprises stretching 25 a yarn having a basis of an organic derivative of cellulose by at least 40% of its original length by passing it through hot water at a temperature of at least 95° C. during its travel between feed and take-up devices which insert a low twist in 30 the yarn, the stretching and twisting of the yarn being effected in the actual presence of the hot water.

3. Process for the production of low twist yarn of improved tenacity, which comprises stretching 35 a yarn having a basis of an organic derivative of cellulose by at least 40% of its original length by passing it through wet steam at a temperature of at least 95° C. during its travel between feed and take-up devices which insert a low twist in 40 the yarn, the stretching and twisting of the yarn being effected in the actual presence of the wet steam.

4. Process for the production of low twist 45 yarn of improved tenacity, which comprises stretching a yarn having a basis of cellulose acetate by at least 40% of its original length by passing it through wet steam at a temperature of at least 120° C. during its travel between feed and take-up devices which insert a low twist in 50 the yarn, the stretching and twisting of the yarn being effected in the actual presence of the wet steam.

5. Process for the production of low twist 55 yarn of improved tenacity, which comprises stretching a yarn having a basis of cellulose acetate by at least 40% of its original length by passing it through hot water at a temperature of at least 120° C. during its travel between feed and take-up devices which insert a low twist in 60 the yarn, the stretching and twisting of the yarn being effected in the actual presence of the hot water.

HENRY DREYFUS.

ROBERT WIGHTON MONCRIEFF.

FRANK BRENTNALL HILL.